

Aug. 22, 1939.

E. FRIEDERICH ET AL

2,170,683

ELECTRIC INCANDESCENT LAMP

Filed March 18, 1936



Inventors:  
Ernst Friederich,  
Wilfried Meyer,  
by Harry E. Dunham  
Their Attorney.

## UNITED STATES PATENT OFFICE

2,170,683

## ELECTRIC INCANDESCENT LAMP

Ernst Friederich, Berlin-Charlottenburg, and Wilfried Meyer, Birkenthaler, near Berlin, Germany, assignors to General Electric Company, a corporation of New York

Application March 18, 1936, Serial No. 69,591  
In Germany April 30, 1935.

5 Claims. (Cl. 176—19)

Our invention relates to electric incandescent lamps and more particularly to incandescent bodies or filaments for such lamps.

In the conventional incandescent lamps having tungsten filaments, the current densities are much higher upon switching in of the lamps than they are during the subsequent normal burning of the lamps. This is not harmful to the incandescent lamp itself since the filament is not heated to a temperature in excess of that attained during the normal burning of the lamp. However, this characteristic may be harmful, for instance, in cases where the lamps are operated in series with other current consuming devices, the starting time of which exceeds that of the filament of the lamp. In such cases the voltage drops a few seconds, or even minutes, after the switching in of the lamp is frequently greater than the drop existing during the normal operation of the lamp, thereby causing a much higher watt consumption and considerable overheating which, in turn, shortens the life of the lamp.

An object of our invention is to provide an incandescent body or filament having a higher thermal capacity, that is, a longer heating period than that of the ordinary tungsten filament and of the other filaments which have since become known. Another object is the provision of a lamp which may be used in series with other power consuming devices, such as lamps for the illumination of dials, of instruments, lamps for microscopes, etc., where tungsten filament lamps may not be used unless special protective measures are taken.

The drawing is a perspective view of an incandescent lamp comprising our invention.

Referring to the drawing, the lamp comprises a glass bulb or envelope 10 having a pair of lead-in wires 11—11 sealed therethrough and supporting an incandescent body or filament 12 comprising a rare metallic oxide.

According to our invention, a number of substances are suitable for the incandescent bodies, especially uranium dioxide and some of the lower vanadium oxides, niobium oxides and titanium oxides. Some of the said lower oxides, especially the lower oxides of vanadium and niobium, as well as those of titanium, have such a low specific resistivity that incandescent bodies made therefrom may have the thickness of a metal thread. These oxides are preferably mixed with insulators which permit a complete or partial solution of the conducting ingredient in the non-conducting vehicle, such as a low titanium oxide in magnesium oxide. Because of the mutual solution, it

is possible to proceed independently of the original grain size of the materials and a large number of filaments may be manufactured having the same electrical properties. Instead of magnesium oxide, other insulating oxides may be used, such as aluminum oxide, chromium oxide, manganese oxide, etc. As a result of the mixing or solution, the specific resistivity of the filament is so increased that filaments may be produced having a comparatively large diameter, that is, a comparatively high thermal capacity for a given length.

Incandescent bodies made of oxides and oxide mixtures and of considerable thickness have been proposed heretofore for use in the so-called Nernst lamp. These bodies, however, have the disadvantage that they must be preheated by a special appliance in order to render them conductive. The incandescent bodies according to the present invention are conductive at low voltages and have, unlike the Nernst lamp, a purely electronic conductivity. These bodies must be operated in an evacuated space, for otherwise they would oxidize into non-conducting or poorly conducting oxides, such as  $TiO_2$ ,  $V_2O_5$ ,  $Nb_2O_5$ ,  $V_3O_8$ .

It has been found that at very high temperatures, above, say  $1200^{\circ} C.$ , the loosening of the lattice system of oxides becomes so pronounced that even those bodies which at room temperature have a perfect electronic conductivity are partly electrolytically decomposed at the said higher temperatures. It has been observed that these oxides retain their electronic conductivity completely, even at temperatures up to  $2000^{\circ} C.$  and more, when a small partial pressure of oxygen is provided. Of course this partial pressure of oxygen must be so slight that the incandescent body will not oxidize to a higher state of the oxide. It is particularly advantageous to fill the envelopes or bulbs of the lamps with nitrogen to which is added 0.001% to 0.5% of oxygen. Other inert gases may of course be used in place of nitrogen. Hydrogen may also be used as a gas filling when the incandescent bodies are made of uranium dioxide, and in that case the slightly oxidizing atmosphere is created by adding water vapor to the hydrogen. The lamps may also be made without an inert gas and having only a slight oxygen content. The incandescent bodies may be made in the conventional manner by pressing or extrusion with or without binders, and by baking at high temperatures. They may also be provided with coatings of selectively radiating or poorly radiat-

ing substances such as magnesia, thorium dioxide and zirconium dioxide.

What we claim as new and desire to secure by Letters Patent of the United States is:

5. 1. An electric incandescent lamp comprising an envelope, an incandescent body in said envelope comprising a rare oxidizable metallic oxide which is conductive at ordinary temperatures, and an atmosphere comprising a small amount of 10 oxygen in said envelope, the amount of oxygen being sufficient to cause said incandescent body to retain its electronic conductivity at temperatures of the order of 2000° C. but insufficient to cause conversion of said rare metallic oxide to a higher form of non-conductive oxide.
15. 2. An electric incandescent lamp comprising an envelope, an incandescent body in said envelope comprising a rare oxidizable metallic oxide which is conductive at ordinary temperatures, and an atmosphere comprising an inert gas and a small 20 amount of oxygen in said envelope, the amount of oxygen being sufficient to cause said incandescent body to retain its electronic conductivity at temperatures of the order of 2000° C. but insufficient to cause conversion of said rare metallic oxide to a higher form of non-conductive oxide.
25. 3. An electric incandescent lamp comprising an envelope, an incandescent body in said envelope comprising a mixture of a rare oxidizable metallic oxide which is conductive at ordinary temperatures and a non-conductive refractory metallic oxide, and an atmosphere comprising a small 30 amount of oxygen in said envelope, the amount

of oxygen being sufficient to cause said incandescent body to retain its electronic conductivity at temperatures of the order of 2000° C. but insufficient to cause conversion of said rare metallic oxide to a higher form of non-conductive oxide. 5

4. An electric incandescent lamp comprising an envelope, an incandescent body in said envelope comprising a mixture of a rare oxidizable metallic oxide which is conductive at ordinary temperatures and a non-conductive refractory metallic oxide, and an atmosphere comprising an inert 10 gas and a small amount of oxygen in said envelope, the amount of oxygen being sufficient to cause said incandescent body to retain its electronic conductivity at temperatures of the order of 2000° C. but insufficient to cause conversion of said rare metallic oxide to a higher form of non-conductive oxide. 15

5. An electric lamp comprising a sealed envelope and a filament in said envelope consisting of a mixture of an oxide of the group of metals uranium, vanadium, niobium and titanium which is conductive at ordinary temperatures and a non-conductive refractory oxide, said envelope containing an atmosphere comprising a small 20 quantity of oxygen sufficient to cause said filament to retain its electronic conductivity at temperatures of the order of 2000° C. but insufficient to cause conversion of said first-mentioned oxide to a higher form of non-conductive oxide. 25

ERNST FRIEDERICH.  
WILFRIED MEYER.